

## UNITED STATES PATENT OFFICE

2,370,648

## NONCAKING FLATTING AGENT

Earl K. Fischer, Long Island City, N. Y., assignor  
to Interchemical Corporation, New York, N. Y.,  
a corporation of Ohio

No Drawing. Application December 12, 1941,  
Serial No. 422,683

4 Claims. (Cl. 260—71)

This invention relates to the preparation of dull or flat coating compositions containing as the flattening agent insoluble carbamide-aldehyde resin powders, and it is particularly directed to a method for treating these powders so as to make them easily dispersible.

It is often desired to obtain finishes which are more or less matte, either for the decorative or for the frequently desirable optical effect. The trade in general has adopted, as flattening agents, powders which are relatively insoluble in the coating compositions and which can be dispersed therein to yield films which are dull or flat because of the fact that the insoluble flattening agent scatters the incident light. Where a flattening agent is desired which may be incorporated in any of the standard coating compositions in large quantity without materially detracting from physical properties of the finished film, powders of the insoluble carbamide-aldehyde resins have been developed, particularly the insoluble urea-formaldehyde resins, and these form the subject matter of co-pending application Serial No. 407,623, filed August 20, 1941, in the name of Loy S. Engle.

Although these carbamide-aldehyde resin flattening agents (hereinafter referred to as "urea flattening agents") are outstanding in their flattening abilities and minimize the effects of abrasion, they are sometimes difficult to disperse permanently in the conventional vehicles. When they have been dispersed in the vehicles and have been allowed to stand, as in storage, they settle out in the form of fairly hard cakes which are not redispersible without regrinding, and which do not give the expected flattening on application.

This invention provides a treatment whereby these urea resin flattening agents may settle out, if at all, in the form of soft or curdy deposits which are easily redispersible in the vehicle by simple stirring. The invention also includes the treated urea resin flattening agents and finishing compositions containing the same.

I have found that the urea flattening agents will not settle out into hard cakes after dispersion in conventional vehicles if they are in a flocculated condition. The resin particles may be treated prior to, or during, incorporation in the vehicle in a way which causes them to flocculate, and this treatment consists in depositing an extremely fine film of a polar liquid on the surfaces of the particles. This is most easily done by bringing the resin particles into intimate contact with the polar liquid prior to introduction into the vehicle, and it is preferred to grind the powder and liquid on a roll mill to form a paste

or mealy mass and to stir this mass into the vehicle.

Although all polar liquids will have some flocculating effect on the resin particles, the more highly polar liquids are more effective, provided, of course, the liquid is not so chemically reactive that it will attack the particles themselves or materially alter their physical and chemical properties. Also, for most coating formulations it is desirable that the flocculating liquid be sufficiently volatile that it will be expelled from the coating during baking or other drying operations. I have found that the polar liquids which are most satisfactory for this purpose are those which may be broadly classed as polyhydroxy compounds, and three especially satisfactory compounds of this class are ethylene glycol, glycerol and triethanolamine. Water can be used in some cases, but usually it is necessary for other reasons to avoid the presence of much water in the finishing composition. Of course, mixtures of two or more of these liquids may be used.

A comparison was made between the settling characteristics and re-dispersibility of an insoluble urea-formaldehyde powder in three different types of finish, both when treated with various polar liquids and when untreated. The urea resin powder was ground on a three-roll mill with an equal weight of the polar liquid, and the paste thus obtained was stirred into the finish and allowed to settle by standing for 20 days. The three finishes were as follows:

(A) A varnish containing an oil soluble phenolic resin, China-wood oil varnish and 50% hydrocarbon solvent.

(B) A urea-alkyd baking finish containing 65% solvent comprising toluene and butanol.

(C) A nitrocellulose lacquer base thinned with ester solvents to spraying consistency.

In finish A the untreated resin powder settled into a firm gel which was very difficultly redispersible. On the other hand, the resin powder which had been wet with polar liquids, especially hydroxy compounds (e. g., water, ethylene glycol, glycerol, butanol, octanol, diethanolamine, triethanolamine, ethyl lactate, etc.) settled into soft masses which were readily redispersible by simple stirring.

In finish B the untreated resin powder settled into a tough solid which could not be redispersible by stirring, whereas the resin powder which had been wet with a polar liquid could be redispersible. However, with this finish not all of the polar liquids were equally satisfactory. The mono-hydroxy compounds which were so successful

with finish A permitted the powder to settle into rather compact resin cakes which required vigorous stirring for redispersion. On the other hand, the polyhydroxy compounds, such as ethylene glycol, glycerol and the polyalkylolamines (e.g., the di- and tri-ethanolamines) yielded soft resin cakes which were easily redispersed.

In finish C the untreated resin powder settled to a tough solid in the same way as with finish B. However, the resin powders which had been wet with polar liquids were not all easily redispersed. Those powders which were wet with liquids having less than two hydroxyl groups settled into such hard and compact cakes in this finish that they were redispersed only with difficulty after prolonged, vigorous stirring, whereas those urea resin powders which were wet with polyhydroxy compounds settled to soft flocs or curds which were easily redispersed. Especially suitable liquids were ethylene glycol, glycerol and the polyalkylolamines.

These treated urea resin flattening agents may be used in finishes in many different ways, a few of which are described in the following examples by way of illustration.

*Example 1—(Matte-finish black baking enamel)*

A urea resin flattening agent is thoroughly wet with an equal weight of ethylene glycol by grinding on a three-roll mill. Four passes at a relatively loose roll setting provide the necessary wetting. A matte-finish, synthetic black baking enamel may be formulated as follows:

| Per cent by weight               |       |
|----------------------------------|-------|
| Carbon black, high color         | 1.5   |
| Urea resin, 50% in butanol       | 36.0  |
| Alkyd resin, 50% in xylene       | 36.0  |
| Above described flattening paste | 15.0  |
| Butanol                          | 3.0   |
| Toluene                          | 8.5   |
|                                  | 100.0 |

This composition is suitable for spray application by further dilution with 25% of a solvent mixture containing four parts of toluene to one part of butanol.

*Example 2—(Dull finish printing ink)*

A dull finish printing ink may be prepared by dispersing carbon black in linseed oil varnish in conventional manner by five passes on a three-roll ink mill, in the following ratios:

| Per cent by weight                       |       |
|------------------------------------------|-------|
| Carbon black, ink grade                  | 19.0  |
| Bodied linseed oil (No. 1 Gardner-Holdt) | 65.0  |
| Then add—                                |       |
| Cobalt linoleate drier                   | 6.0   |
| Flattening paste from Example 1          | 10.0  |
|                                          | 100.0 |

This mixture is given two loose passes on the roll mill.

*Example 3—(Matte varnish for brush application)*

A matte finish varnish for brush application may be formulated from a conventional varnish by addition of a urea resin flattening paste prepared by grinding, as described in Example 1, a urea resin flattening agent with glycerol in equal proportions. In this case a phenolic modified drying oil varnish was used, which gave a break-

down formulation of the final product as follows:

|                                         | Per cent by weight |
|-----------------------------------------|--------------------|
| 100% phenolic resin-tung oil complex    | 30                 |
| Linseed oil (boiled)                    | 10                 |
| Urea resin in glycerol flattening paste | 15                 |
| Turpentine                              | 5                  |
| Mineral spirits                         | 40                 |
|                                         | 100                |

Besides the organic liquids specifically mentioned, other polar liquids may be successfully used for the purpose described, although the polyhydroxy liquids are generally superior to others. Although water itself is a good flocculating agent for the insoluble urea resin flattening powders, its use is limited because it may cause blushing of the coated films, cause an undesirable thickening, or otherwise detrimentally affect the finish.

About 5% of flocculating agent, based on the weight of the condensation product, is generally required to produce the desired results.

The preferred method of coating the resin particles with the polar liquid is, of course, to bring the two into intimate contact before incorporation in the finish or vehicle. However, it is possible (and sometimes practical) to wet the resin powder after it has been dispersed in the vehicle or finish, simply by adding the polar liquid to the finish and intimately dispersing it by milling or otherwise thoroughly agitating the mixture.

I claim:

1. A finishing composition which dries to a flat surface, comprising an organic film-forming composition which normally dries to a glossy film, said composition having dispersed therein a substantially insoluble carbamide aldehyde condensation product in finely divided form to produce the flat drying properties, the particles of condensation product being coated with at least 5%, based on the weight of condensation product, of a flocculating agent therefor comprising an organic liquid containing an alcoholic hydroxyl group.

2. A finishing composition which dries to a flat surface, comprising an organic film-forming composition which normally dries to a glossy film, said composition having dispersed therein a substantially insoluble carbamide aldehyde condensation product in finely divided form to produce the flat drying properties, the particles of condensation product being coated with at least 5%, based on the weight of condensation product, of a flocculating agent therefor comprising a polyhydric alcohol.

3. A flattening agent useful in the production of flat organic finishing compositions consisting essentially of a substantially insoluble carbamide aldehyde condensation product in finely divided form, the particles of condensation product being coated with at least 5%, based on the weight of condensation product, of a flocculating agent therefor comprising an organic liquid containing an alcoholic hydroxyl group.

4. A flattening agent useful in the production of flat organic finishing compositions consisting essentially of a substantially insoluble carbamide aldehyde condensation product in finely divided form, the particles of condensation product being coated with at least 5%, based on the weight of condensation product, of a flocculating agent therefor comprising a polyhydric alcohol.

EARL K. FISCHER.